

# UNITED STATES PATENT OFFICE.

SYDNEY J. NEWSHAM, OF NEW YORK, N. Y., ASSIGNOR OF ONE-HALF TO  
FRANCIS T. SARGENT, OF SAME PLACE.

## ART OF STAINING OR ENAMELING GLASS, &c.

SPECIFICATION forming part of Letters Patent No. 256,916, dated April 25, 1882.

Application filed October 1, 1880. Renewed December 23, 1881. (No specimens.)

*To all whom it may concern:*

Be it known that I, SYDNEY J. NEWSHAM, of the city, county, and State of New York, have invented certain new and useful Improvements in the Art of Staining or Enameling Glass and Similar Material, of which the following is a specification.

My invention relates to the application of stains or enamels to the surface of flat glass or other articles made of glass, china, porcelain, earthenware, &c., whether the parts to be stained have been previously etched or eaten away or not; and the object of my invention is to effect the enameling or staining operation with or without previous etching, in a cheaper and more easy manner, and with a more perfect result than heretofore attained, as herein-after fully set forth.

To carry out my invention, the article to be stained or enameled is, by preference, first etched in the usual manner—that is, the desired ornament or design is first produced on its surface by the well-known process of transferring or printing, or in any other of the usual modes of preparing the surface for etching—whereby the parts desired to be etched and stained are left exposed, while the remainder is protected by a suitable protecting ink, varnish, or other material, after which preparation the etching is effected in the usual manner by exposure to etching-acid or a mixture of such acids. The enamel or stain, which is, of course, composed of some vitrifiable color, is also prepared in the usual manner, being mixed or ground with water into the condition of a paint or thin paste, which can be applied with a brush. Heretofore, however, after the etching has been made, the protective ink or other substance has been immediately removed from the "ground," thus leaving the entire surface exposed, and the enamel or stain is then applied to the etched or sunken parts, all the features and intricacies thereof being carefully followed with the brush, so as to fill in the same with the stain, and avoid overrunning the edges of the ground therewith as much as possible, after which the enamel or stain is fused and fixed by baking in a furnace in the well-known manner. It may be observed, however, that the brushing in of the enamel

or stain under the above conditions has to be conducted carefully, is laborious, requires considerable time, and demands skilled hands. Even then it is not always possible to confine the stain to the etched lines and avoid overrunning into the ground, and of course when the article is submitted to the heat of the furnace, these overrunnings will become fused and fixed, producing defects in the design; or, again, if any overplus of stain exists in the etched lines themselves, there is nothing to restrain this overplus when fused from overflowing the etched lines and producing the effect of blurred and imperfect lines.

Now, according to my improvement, after the etching has been effected I allow the protective ink or etching-ground to remain undisturbed, and simply remove the deposit of silica dissolved by the etching-acid by means of a soft brush wet with water, so as to thoroughly clean out the lines of the etching, yet leave the protective ground intact. I then brush the stain over the surface, so as to properly fill the lines or cavities of the etching. This may, of course, be done quite quickly and carelessly by a few bold strokes with a large brush, there being no necessity to trace the intricacies of the design or to specially avoid overrunning the inky ground here and there with traces of the stain, and hence no skilled hands are required for this operation. After the enamel or stain is thus applied the article may now be placed in the furnace, the heat of which will, of course, first evaporate the moisture of the enamel, and the volatile matter of the protecting-ink, thus finally drying and hardening the ink around the etched and enameled lines. Hence when the enamel becomes fused it is confined sharply to the etched lines by the hardened ink surrounding it, which prevents the spread or overflowing of the enamel beyond the etched lines of the design, so that sharp, distinct, and perfect designs may be thus obtained. When the article is removed from the furnace its surface may be finally cleaned, so as to remove the dry and calcined ink by brushing off the same with a stiff brush, either dry or wet with water, thus completing the process, and it may be readily observed that the ink is much more easily removed at this stage than it would be directly after the

etching; as has been heretofore done, as it is then soft and requires to be dissolved off with benzine or turpentine, which is, of course, more expensive and laborious, whereas by my system it is reduced to the condition of a charred crust, which is readily brushed off, leaving the surface clean and bright.

In most cases, after the enamel is applied, as above described, but before the article is placed in the furnace, I prefer to cover the whole surface on which the design is to appear with what may be called an "absorbent" coating of some fire-proof absorbent substance or pigment—such as the earth paints ground with water into a stiff paint. This coating I apply with a brush, in as thick a coating as can be conveniently applied with a brush, over the inked ground, but not over the enamel-lines of the design, so as to completely cover and protect the same. As soon as this coating becomes dried by the first heat of the furnace it acts as an absorbent to absorb any of the resinous or waxy matter of the ink that may be liquefied by the heat, thereby preventing the running of the ink, and hence preserving the ground around the etched lines which contain the enamel, so as to effectually confine the enamel thereto and prevent any overflowing thereof onto the ground or over the etched lines, thus enabling perfect work to be secured with more certainty in all cases. By absorbing the liquefiable matter of the inky ground this absorbent coating hence also prevents the strong adhesion of the ink to the surface of the glass or other material operated upon, and thus reduces the whole ground to a brittle crust, which is easily brushed off with a stiff brush after the baking operation, thus leaving the decorated surface of the article quite clean. When the ink used for the etching-ground is quite hard, or contains little liquefiable matter, having little tendency to run, the final absorbent coating may be dispensed with; but I generally find it best to employ this coating in all cases, as its application is very simple, its expense almost nothing, and where it may not

be necessary to prevent the ink from running it always renders the ink more easy to remove at the final operation of cleaning than would otherwise be the case.

It may be observed that by my system the design which is to appear in stain or enamel on the surface of the glass or other material need not always be previously etched, for the stain may be applied directly to the cavities in the inky or protective ground which expose the surface of the glass and form the lines of the design, and may then be fixed by fusing, thus producing the stained design without etching at much less cost. For fine work, however, the previous etching is always preferable, but for cheap work it may be thus dispensed with to great advantage.

What I claim is—

1. The improvement in the art of decorating glass or similar material with designs in stains or enamels, consisting in covering the ground with a protective ink or equivalent material, leaving the lines to be decorated exposed, filling in said exposed parts with the stain or enamel, and fusing the same with the protective ground surrounding and confining the enamel, substantially as herein set forth.

2. The herein-described improvement in the art of enameling or staining embossed or etched articles—viz., leaving the protective ground intact after the embossing or etching, then applying the enamel or stain, and baking or fusing the same, with the protective ground surrounding and confining the enamel or stain—substantially as and for the purpose herein set forth.

3. In the art of enameling or staining glass or similar material, the step of covering the protective ground with a coating of an absorbent fire-proof paint previous to the baking or fusing operation, substantially as and for the purpose herein set forth.

SYDNEY J. NEWSHAM.

Witnesses:

EDWARD H. WALES,  
CHAS. M. HIGGINS.